

## 1

3,014,867

**LUBRICATING GREASE WHEREIN THE THICKENER IS THE METAL SOAP OF MIXED ACIDS AND PROCESS FOR FORMING SAME**

Ernest T. Fronezak, Crystal Lake, Ill., assignor to The Pure Oil Company, Chicago, Ill., a corporation of Ohio

No Drawing. Filed July 11, 1957, Ser. No. 671,141  
10 Claims. (Cl. 252—40.5)

This invention relates to grease compositions and to a method for their preparation. More particularly this invention relates to a gelatinous grease composition containing an improved metal-soap gelling agent in a solvent-refined lubricating oil blended with a solvent extract from the manufacture of lubricating oil stocks.

Greases are conventionally considered as gel systems of fluid lubricants, such as mineral lubricating oils or equivalent synthetic lubricating oils, and gelling agents, such as metal soaps or equivalent inorganic non-soap gelling agents. The most common greases are soap-thickened greases which are normally prepared by saponification of fats in mineral oil, followed by dehydration and dilution with mineral oil to the desired consistency. In the manufacture of greases, the highest consideration is given to obtaining of satisfactory physical properties of melting point, consistency (as measured by the cone penetration test), shear stability (as measured by change in worked consistency), free acid or alkali content, and stability in storage and use. In the economics of grease-making the yield of grease is extremely important. The yield of grease is ordinarily defined as the relative amount of grease made from a unit amount of gelling agent which will produce greases of the same consistency. Thus, if 10% of one soap is required to produce a No. 2 grease and 15% of another soap is required to produce a No. 2 grease, the former grease is produced in much higher yield. Since greases are made from lubricating oil stocks, it is desirable to make greases from the cheaper solvent-refined lubricating oils. However, it has been found that grease compositions prepared from solvent-refined lubricating oil stocks require a much higher proportion of soap (and are thus produced in lower yield) than the more expensive distilled lubricating oils. Since the soap represents a relatively high proportion of the cost of a grease, it is very desirable that greases be prepared which use very small amounts of soap and which may use the inexpensive solvent-refined lubricating oils.

One of the objects of this invention is to provide a grease composition containing a metal-soap gelling agent.

Another object of this invention is to provide a very high yield grease using an improved metal-soap gelling agent.

A further object of this invention is to provide an improved grease in high yield utilizing a solvent-refined lubricating oil base.

A further object of this invention is to provide an improved grease in which the lubricating oil base is composed of a mixture of solvent-refined lubricating oils and a solvent-extract from lubricating oil fractions.

A feature of this invention is the provision of an improved grease utilizing as the gelling agent a metal soap of mixed acids which are obtained as the volatile fraction from the vacuum distillation at 200°—270° C. and 4—20 mm. pressure of the by-product acids obtained in the preparation of sebacic acid from castor oil by treatment with alkali.

## 2

Another feature of this invention is the provision of an improved grease which utilizes as the mineral lubricating oil base a solvent-refined lubricating oil, alone or in mixture with the solvent-extract from lubricating oil fractions, gelled by an alkali metal soap of the volatile fraction of the by-product acids obtained in the preparation of sebacic acid from castor oil by treatment with alkali.

Other objects and features of this invention will become apparent from time to time throughout the specification and claims as hereinafter related.

This invention is based upon the discovery that greases may be prepared in high yield from lubricating oils and a gelling agent which consists of a metal soap of the mixed acids which are obtained as the volatile fraction from the vacuum distillation at 200°—270° C. and 4—20 mm. pressure of the by-product acids obtained in the preparation of sebacic acid from castor oil by treatment with alkali. These metal soaps produce satisfactory greases with any lubricating oil base but have been found unexpectedly to produce very high yields from lubricating oil bases which consist of solvent-refined lubricating oils, alone, or in combination with solvent-extracts from lubricating oil fractions.

In the manufacture of greases according to this invention, the gelling agents used consist of metal soaps of mixed acids which are by-products from the manufacture of sebacic acid from castor oil. These mixed acids are prepared according to a process described in Cheetham et al., U.S. Patent 2,267,269, the process for which will be described more fully hereinafter, and are referred to hereinafter throughout the specification and claims as mixed acids I. Sebacic acid is made commercially by fusing castor oil with caustic alkali, or (as described in Patent 2,182,056) by heating the two in the presence of water under high pressure. The initial reaction products are octanol-2, methyl-hexyl ketone, the sodium salt of sebacic acid, and the sodium salts of various by-product acids formed by side reactions. The octanol-2 and methyl-hexyl ketone are removed by distillation. The acids formed by side reactions are separated by dissolving the residue in water and acidifying the same with a mineral acid to cause a separation into a lower aqueous layer and an upper oily layer. The lower layer, which is an aqueous solution of sodium sebacate, is drawn off and acidified to precipitate the sebacic acid. The upper oily layer contains the by-product acids formed by side reactions. The by-product acids are separated by distillation at low pressures. These acids are subjected to a temperature of about 100° to 200° C. and 20 mm. pressure for removal of the more volatile acid materials. The mixture is then subjected to progressively increasing temperatures between 200° and 270° C. and a pressure gradually reduced from 20 mm. to about 4 mm. At temperatures between 200° and 270° C. and pressures of 4—20 mm. a distillate is obtained which constitutes about 40% of the by-product acids. This distillate consists of a mixture of fatty acids, both saturated and unsaturated, of very uncertain composition, which is referred to in the specification and claims as mixed acids I. Mixed acids I consist of a very complex mixture of fatty acids containing from 11 to 18 carbon atoms per molecule, including both saturated and unsaturated acids. Among the unsaturated acids there are some with cis configurations and some with trans configurations. The exact analysis of the

composition has never been completely worked out and the composition has never been reproduced by a synthetic mixture of fatty acids because of its complexity and

because of the somewhat unique combination of titre, acid value and iodine value. Mixed acids I contain about 15%  $C_{11-13}$  acids, about 25%  $C_{14-15}$  acids and about 60%  $C_{16-18}$  acids. These mixed acids have the following properties:

|                                               |       |         |
|-----------------------------------------------|-------|---------|
| Titre                                         | 0° C. | 35-38   |
| Iodine value                                  |       | 36-42   |
| Fatty acid (calculated as percent oleic acid) |       | 112-115 |
| Acid value                                    |       | 220-256 |
| Saponification value                          |       | 221-227 |
| NPA color                                     |       | 1½      |

Mixed acids I which were used in the formulation of greases according to this invention are obtainable from Harchem Division of Wallace and Tiernan Inc. under the trade name "CD-N" acids.

In preparing greases in accordance with this invention the following ranges of starting materials are preferred:

|                                                              | Percent  |    |
|--------------------------------------------------------------|----------|----|
| Mixed acids I                                                | 3-20     | 20 |
| Metallic hydroxide                                           | 0.75-5.0 |    |
| Solvent extract from production of high V.I.<br>bright stock | 6-12     |    |
| Solvent-refined 200 vis. neutral oil                         | 65-85    |    |
| Coupling agent                                               | 0.3-6.0  |    |

The mixed acids I are as previously defined. The metallic hydroxide may be any alkali metal hydroxide, such as NaOH, LiOH, or KOH, or alkaline earth metal hydroxide, such as Ca(OH)<sub>2</sub>, Mg(OH)<sub>2</sub>, or Ba(OH)<sub>2</sub>, but is preferably sodium hydroxide. In this composition any suitable bright stock extract or neutral oil may be used, dependent only upon the economic factors in making the grease and the type of grease desired. A satisfactory grease may also be prepared using solvent-refined oils without any solvent-extract, or using distilled lubricating oils. The coupling agent may be any conventional grease coupling agent, such as glycerol, ethylene glycol or other liquid glycols, or liquid polyethylene glycols.

In preparing a grease from the above ingredients, the acids, coupling agent, bright stock extract, and about 20% of the solvent-refined neutral oil are charged to a grease-making kettle and heated to 120°-130° F., with agitation. When the mixture has reached a temperature of 120°-130° F. the metal hydroxide is added as a 35-40% solution in water. The batch is gradually heated to a temperature of 210°-220° F. to complete the neutralization of the acids and to evaporate part of the water. The temperature of the batch is then increased to 320°-340° F. for a time sufficient to complete the dehydration of the grease composition. After the evaporation of water from the grease mixture is completed, the grease is cut to any desired soap concentration by adding the remainder of the solvent-refined neutral oil. The diluted grease mixture is then cooled to 180°-190° F. and homogenized in a colloid mill or other suitable shearing device to produce a smooth, fine-textured grease.

The utility and superior properties of greases produced according to this invention are illustrated by the following examples, which, however, should not be considered as limiting the grease compositions to those specifically described.

#### Example 1

A grease was prepared according to this invention from the following ingredients in the proportions indicated:

| Component:                        | Proportion (wt. percent) |
|-----------------------------------|--------------------------|
| Mixed acids I                     | 4.17                     |
| Sodium hydroxide                  | 0.88                     |
| Bright stock extract <sup>1</sup> | 10.01                    |
| 200 vis. neutral oil <sup>2</sup> | 83.90                    |
| Carbowax 1500 <sup>3</sup>        | 1.04                     |

<sup>1</sup> The bright stock extract used is a highly aromatic oil of high viscosity. It is obtained as the phenol extract from the production of solvent-refined high V.I. bright stock and has the following physical and chemical properties:

|                                   |          |
|-----------------------------------|----------|
| Physical:                         |          |
| API gravity                       | 14       |
| Specific gravity, 60° F.          | 0.973    |
| Pounds/gallon                     | 8.100    |
| SUS viscosity:                    |          |
| @ 100° F.                         | 27,000   |
| @ 150° F.                         | 2,447    |
| @ 210° F.                         | 369      |
| NPA color                         | 5 dilute |
| Flash, ° F.                       | 530      |
| Pour, ° F.                        | 65       |
| Percent volatile 3 hrs. @ 325° F. | 0.06     |

|                     |       |
|---------------------|-------|
| Chemical:           |       |
| Percent aromatics   | 90    |
| Percent asphaltenes | Ni1   |
| Aniline point, ° F. | 149.5 |

|                                |      |
|--------------------------------|------|
| Rostler analysis:              |      |
| Percent nitrogen bases         | 4.3  |
| Percent group 1 acidifins      | 23.3 |
| Percent group 2 acidifins      | 58.9 |
| Percent saturated hydrocarbons | 13.5 |

<sup>2</sup> The neutral oil used was a 200 SUS at 100° F., solvent-refined neutral oil having the following properties:

|                           |              |
|---------------------------|--------------|
| API gravity               | 29.5         |
| Flash                     | 400° F. min. |
| Fire                      | 465° F. min. |
| Viscosity, SUS at 100° F. | 200          |
| Pour                      | 0° F.        |
| Color NPA                 | 3 max.       |
| Carbon residue            | 0.05% max.   |
| Sulfur                    | 0.45% max.   |
| Ash                       | 0.01% max.   |
| Neutralization number     | 0.1 max.     |
| Viscosity index           | 90 min.      |

<sup>3</sup> Carbowax 1500 is a polyethylene glycol produced by Carbowax and Carbon Chemicals Company consisting of a mixture of polyethylene glycols of the general formula  $HOC_2H_4(OCH_2H_4)_nOH$ , and having an average molecular weight between 500 and 600.

In preparing this grease the mixed acids I, bright stock extract, Carbowax 1500, and about 20% of the solvent-refined neutral oil were charged to the grease-making kettle and heated to about 120°-130° F., with agitation. When the temperature of the mixture reached 120°-130° F. the sodium hydroxide was added as a concentrated solution (about 35-40% concentration). The temperature of the batch was increased first to a temperature of about 210°-220° F. to complete neutralization of the acids and to evaporate part of the water, and then to about 320°-340° F. to complete evaporation of the water from the grease mixture. After the grease mixture was completely dehydrated, the remainder of the natural oil was added to cut the soap concentration to a predetermined desired level. The diluted grease mixture was then cooled to 180°-190° F. and homogenized in a colloid mill (a Marco Kom-Bi-Nator) to produce a smooth, fine-textured grease. The grease produced from these components, utilizing this method of compounding, was a No. 0 grease having an unworked penetration of 352 and a worked penetration of 351. The consistency of this grease is very unusual and excellent for the soap concentrations employed. The narrow spread between worked and unworked penetrations is particularly noteworthy since it is indicative of the excellent shear or consistency stability of the grease.

#### Example 2

When a grease is prepared using the components of Example 1 in the same proportion but substituting ethylene glycol or glycerol for the Carbowax 1500, in the same proportion, No. 0 greases are obtained in each case which have a narrow range of unworked and worked penetrations as in Example 1.

#### Example 3

Another grease was prepared from the following ingredients, in the proportion indicated:

| Component:                                                       | Concentration (wt. percent) |
|------------------------------------------------------------------|-----------------------------|
| Mixed acids I                                                    | 8.92                        |
| Sodium hydroxide (as concentrated aqueous solution)              | 1.62                        |
| Bright stock extract (as defined in Example 1)                   | 8.84                        |
| 200 vis. solvent-extracted neutral oil (as defined in Example 1) | 79.68                       |
| Glycerol                                                         | 0.89                        |

<sup>70</sup> This grease was prepared by the identical procedure used

in Examples 1 and 2, with the glycerol being added at the same point in the processing in place of the Carbowax 1500. A No. 2 grease was obtained which had an unworked penetration of 273 and a worked penetration of 290. As in the case of Examples 1 and 2, the grease obtained is in unexpectedly high yield and has a narrow range of worked and unworked penetration, indicative of high shear or consistency stability.

*Example 4*

In still another experiment a grease was prepared using conventional soap stock or fat to illustrate the problems encountered in preparing greases from solvent-refined oils with conventional grease-making soaps. This grease was prepared from the following components in the proportions indicated:

| Component:                                                     | Concentration (wt. percent) |
|----------------------------------------------------------------|-----------------------------|
| Beef tallow                                                    | 6.42                        |
| Hydrogenated fish oil                                          | 6.42                        |
| Sodium hydroxide (in 35% aqueous solution)                     | 2.07                        |
| 200 vis. solvent-refined neutral oil (as defined in Example 1) | 16.98                       |
| 350 vis. solvent-refined neutral oil <sup>1</sup>              | 68.11                       |

<sup>1</sup> This oil was a solvent-refined neutral oil produced by phenol extraction of lubricating oil stocks and having the following properties:

|                           |              |
|---------------------------|--------------|
| API gravity               | 30.5         |
| Flash                     | 460° F. min. |
| Fire                      | 510° F. min. |
| Viscosity, SUS at 100° F. | 350          |
| Pour                      | 0° F. max.   |
| Color NPA                 | 2            |
| Carbon                    | 0.03% max.   |
| Ash                       | 0.01% max.   |
| Sulfur                    | 0.30% max.   |
| Viscosity index           | 100 min.     |

This grease was prepared using standard, open-kettle procedure for preparation of soda greases, with the glycerol coupling agent being produced in situ by the saponification of the fats. The grease which was prepared in this manner is typical of greases prepared from solvent-refined lubricating oils with conventional grease-making soaps. This grease had an unworked consistency of 278 and a worked consistency of 315, corresponding to a No. 1 grease. The yield of this grease was very poor compared to the greases produced in Examples 1 to 3. The difference between the unworked and worked penetration indicates a poor shear or consistency stability and continued working of the grease in service, or in a homogenizer, would reduce the grease to a very soft or even fluid product.

*Example 5*

When a grease is prepared in accordance with Example 4 using a mineral oil base consisting of a mixture of bright stock extract and 200 vis. solvent-refined neutral oil, in the proportions indicated in Example 2, a grease is obtained which has an unworked consistency corresponding to a No. 0 grease but which degenerates upon working into a fluid product.

*Example 6*

When a grease is prepared using the procedures described in Examples 1 to 3 with a mineral oil base consisting of 200 vis. solvent-refined neutral oil and 350 vis. solvent-refined neutral oil in the proportions indicated in Example 4, but using the sodium soap of mixed acids I, and glycerol as a coupling agent, a stable, No. 3 grease is obtained.

It has been found that satisfactory greases can be made with any mineral oil base using alkali metal or alkaline earth metal soaps of mixed acids I, together with a glycerol, ethylene glycol, or polyethylene glycol coupling agent. It has also been found that while the sodium soaps of mixed acids I produce excellent greases with ordinary mineral oil bases, these soaps are of unexpected utility in preparing greases from the cheaper and more

difficultly gelled solvent-refined oils or mixtures of solvent-refined oils with solvent extracts.

While there have been described several preferred embodiments of this invention, including several specific examples of the best mode of carrying out this invention, it should be understood that within the scope of the appended claims this invention may be practiced otherwise than as specifically described.

What is claimed is:

10. A lubricating grease consisting essentially of a major proportion of a mineral oil selected from the group consisting of solvent-refined lubricating oils and mixtures of solvent-refined lubricating oils with aromatic solvent extracts obtained in the solvent refining of lubricating oils, and a minor proportion of a soap selected from the group consisting of alkali metal soaps and alkaline earth metal soaps of mixed acids I, mixed acids I being obtained as the volatile fraction from the vacuum distillation at 200°-270° C. and 4-20 mm. pressure of
  15. 200 vis. solvent-refined neutral oil (as defined in Example 1) \_\_\_\_\_ 16.98
  20. 350 vis. solvent-refined neutral oil<sup>1</sup> \_\_\_\_\_ 68.11
  25. 30. A grease according to claim 1 in which said soap is present in the mineral oil in a concentration corresponding to the amount of soap produced by neutralization of 3-20% by weight of the composition of mixed acids I with 0.75-5.0% by weight of the composition of a hydroxide of a metal of the group consisting of alkali metals and alkaline earth metals.
  30. 35. A grease according to claim 1 in which said mineral oil is a solvent-refined lubricating oil.
  35. 40. A grease according to claim 2 which includes a coupling agent for said soap and said mineral oil.
  40. 45. A grease according to claim 2 in which said mineral oil is a solvent-refined lubricating oil, said metal hydroxide is sodium hydroxide, and the composition includes a coupling agent of the class consisting of glycerol, ethylene glycol, and liquid polyethylene glycols.
  45. 50. 55. A grease according to claim 2 prepared from the following starting materials:
- |                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                            | Percent  |
|----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|----------|
| Mixed acids I                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                              | 3-20     |
| Metal hydroxide                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                            | 0.75-5.0 |
| 45. Aromatic oil consisting of the solvent extract from production high V.I. bright stock                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                  | 6-12     |
| 200 vis. solvent-refined neutral oil                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                       | 65-85    |
| Coupling agent of the class consisting of glycerol, glycol, and liquid poly-ethylene glycol                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                | 0.3-6.0  |
| 50. 55. 60. 65. 70. 75. 80. 85. 90. 95. 100. 105. 110. 115. 120. 125. 130. 135. 140. 145. 150. 155. 160. 165. 170. 175. 180. 185. 190. 195. 200. 205. 210. 215. 220. 225. 230. 235. 240. 245. 250. 255. 260. 265. 270. 275. 280. 285. 290. 295. 300. 305. 310. 315. 320. 325. 330. 335. 340. 345. 350. 355. 360. 365. 370. 375. 380. 385. 390. 395. 400. 405. 410. 415. 420. 425. 430. 435. 440. 445. 450. 455. 460. 465. 470. 475. 480. 485. 490. 495. 500. 505. 510. 515. 520. 525. 530. 535. 540. 545. 550. 555. 560. 565. 570. 575. 580. 585. 590. 595. 600. 605. 610. 615. 620. 625. 630. 635. 640. 645. 650. 655. 660. 665. 670. 675. 680. 685. 690. 695. 700. 705. 710. 715. 720. 725. 730. 735. 740. 745. 750. 755. 760. 765. 770. 775. 780. 785. 790. 795. 800. 805. 810. 815. 820. 825. 830. 835. 840. 845. 850. 855. 860. 865. 870. 875. 880. 885. 890. 895. 900. 905. 910. 915. 920. 925. 930. 935. 940. 945. 950. 955. 960. 965. 970. 975. 980. 985. 990. 995. 1000. 1005. 1010. 1015. 1020. 1025. 1030. 1035. 1040. 1045. 1050. 1055. 1060. 1065. 1070. 1075. 1080. 1085. 1090. 1095. 1100. 1105. 1110. 1115. 1120. 1125. 1130. 1135. 1140. 1145. 1150. 1155. 1160. 1165. 1170. 1175. 1180. 1185. 1190. 1195. 1200. 1205. 1210. 1215. 1220. 1225. 1230. 1235. 1240. 1245. 1250. 1255. 1260. 1265. 1270. 1275. 1280. 1285. 1290. 1295. 1300. 1305. 1310. 1315. 1320. 1325. 1330. 1335. 1340. 1345. 1350. 1355. 1360. 1365. 1370. 1375. 1380. 1385. 1390. 1395. 1400. 1405. 1410. 1415. 1420. 1425. 1430. 1435. 1440. 1445. 1450. 1455. 1460. 1465. 1470. 1475. 1480. 1485. 1490. 1495. 1500. 1505. 1510. 1515. 1520. 1525. 1530. 1535. 1540. 1545. 1550. 1555. 1560. 1565. 1570. 1575. 1580. 1585. 1590. 1595. 1600. 1605. 1610. 1615. 1620. 1625. 1630. 1635. 1640. 1645. 1650. 1655. 1660. 1665. 1670. 1675. 1680. 1685. 1690. 1695. 1700. 1705. 1710. 1715. 1720. 1725. 1730. 1735. 1740. 1745. 1750. 1755. 1760. 1765. 1770. 1775. 1780. 1785. 1790. 1795. 1800. 1805. 1810. 1815. 1820. 1825. 1830. 1835. 1840. 1845. 1850. 1855. 1860. 1865. 1870. 1875. 1880. 1885. 1890. 1895. 1900. 1905. 1910. 1915. 1920. 1925. 1930. 1935. 1940. 1945. 1950. 1955. 1960. 1965. 1970. 1975. 1980. 1985. 1990. 1995. 2000. 2005. 2010. 2015. 2020. 2025. 2030. 2035. 2040. 2045. 2050. 2055. 2060. 2065. 2070. 2075. 2080. 2085. 2090. 2095. 2100. 2105. 2110. 2115. 2120. 2125. 2130. 2135. 2140. 2145. 2150. 2155. 2160. 2165. 2170. 2175. 2180. 2185. 2190. 2195. 2200. 2205. 2210. 2215. 2220. 2225. 2230. 2235. 2240. 2245. 2250. 2255. 2260. 2265. 2270. 2275. 2280. 2285. 2290. 2295. 2300. 2305. 2310. 2315. 2320. 2325. 2330. 2335. 2340. 2345. 2350. 2355. 2360. 2365. 2370. 2375. 2380. 2385. 2390. 2395. 2400. 2405. 2410. 2415. 2420. 2425. 2430. 2435. 2440. 2445. 2450. 2455. 2460. 2465. 2470. 2475. 2480. 2485. 2490. 2495. 2500. 2505. 2510. 2515. 2520. 2525. 2530. 2535. 2540. 2545. 2550. 2555. 2560. 2565. 2570. 2575. 2580. 2585. 2590. 2595. 2600. 2605. 2610. 2615. 2620. 2625. 2630. 2635. 2640. 2645. 2650. 2655. 2660. 2665. 2670. 2675. 2680. 2685. 2690. 2695. 2700. 2705. 2710. 2715. 2720. 2725. 2730. 2735. 2740. 2745. 2750. 2755. 2760. 2765. 2770. 2775. 2780. 2785. 2790. 2795. 2800. 2805. 2810. 2815. 2820. 2825. 2830. 2835. 2840. 2845. 2850. 2855. 2860. 2865. 2870. 2875. 2880. 2885. 2890. 2895. 2900. 2905. 2910. 2915. 2920. 2925. 2930. 2935. 2940. 2945. 2950. 2955. 2960. 2965. 2970. 2975. 2980. 2985. 2990. 2995. 3000. 3005. 3010. 3015. 3020. 3025. 3030. 3035. 3040. 3045. 3050. 3055. 3060. 3065. 3070. 3075. 3080. 3085. 3090. 3095. 3100. 3105. 3110. 3115. 3120. 3125. 3130. 3135. 3140. 3145. 3150. 3155. 3160. 3165. 3170. 3175. 3180. 3185. 3190. 3195. 3200. 3205. 3210. 3215. 3220. 3225. 3230. 3235. 3240. 3245. 3250. 3255. 3260. 3265. 3270. 3275. 3280. 3285. 3290. 3295. 3300. 3305. 3310. 3315. 3320. 3325. 3330. 3335. 3340. 3345. 3350. 3355. 3360. 3365. 3370. 3375. 3380. 3385. 3390. 3395. 3400. 3405. 3410. 3415. 3420. 3425. 3430. 3435. 3440. 3445. 3450. 3455. 3460. 3465. 3470. 3475. 3480. 3485. 3490. 3495. 3500. 3505. 3510. 3515. 3520. 3525. 3530. 3535. 3540. 3545. 3550. 3555. 3560. 3565. 3570. 3575. 3580. 3585. 3590. 3595. 3600. 3605. 3610. 3615. 3620. 3625. 3630. 3635. 3640. 3645. 3650. 3655. 3660. 3665. 3670. 3675. 3680. 3685. 3690. 3695. 3700. 3705. 3710. 3715. 3720. 3725. 3730. 3735. 3740. 3745. 3750. 3755. 3760. 3765. 3770. 3775. 3780. 3785. 3790. 3795. 3800. 3805. 3810. 3815. 3820. 3825. 3830. 3835. 3840. 3845. 3850. 3855. 3860. 3865. 3870. 3875. 3880. 3885. 3890. 3895. 3900. 3905. 3910. 3915. 3920. 3925. 3930. 3935. 3940. 3945. 3950. 3955. 3960. 3965. 3970. 3975. 3980. 3985. 3990. 3995. 4000. 4005. 4010. 4015. 4020. 4025. 4030. 4035. 4040. 4045. 4050. 4055. 4060. 4065. 4070. 4075. 4080. 4085. 4090. 4095. 4100. 4105. 4110. 4115. 4120. 4125. 4130. 4135. 4140. 4145. 4150. 4155. 4160. 4165. 4170. 4175. 4180. 4185. 4190. 4195. 4200. 4205. 4210. 4215. 4220. 4225. 4230. 4235. 4240. 4245. 4250. 4255. 4260. 4265. 4270. 4275. 4280. 4285. 4290. 4295. 4300. 4305. 4310. 4315. 4320. 4325. 4330. 4335. 4340. 4345. 4350. 4355. 4360. 4365. 4370. 4375. 4380. 4385. 4390. 4395. 4400. 4405. 4410. 4415. 4420. 4425. 4430. 4435. 4440. 4445. 4450. 4455. 4460. 4465. 4470. 4475. 4480. 4485. 4490. 4495. 4500. 4505. 4510. 4515. 4520. 4525. 4530. 4535. 4540. 4545. 4550. 4555. 4560. 4565. 4570. 4575. 4580. 4585. 4590. 4595. 4600. 4605. 4610. 4615. 4620. 4625. 4630. 4635. 4640. 4645. 4650. 4655. 4660. 4665. 4670. 4675. 4680. 4685. 4690. 4695. 4700. 4705. 4710. 4715. 4720. 4725. 4730. 4735. 4740. 4745. 4750. 4755. 4760. 4765. 4770. 4775. 4780. 4785. 4790. 4795. 4800. 4805. 4810. 4815. 4820. 4825. 4830. 4835. 4840. 4845. 4850. 4855. 4860. 4865. 4870. 4875. 4880. 4885. 4890. 4895. 4900. 4905. 4910. 4915. 4920. 4925. 4930. 4935. 4940. 4945. 4950. 4955. 4960. 4965. 4970. 4975. 4980. 4985. 4990. 4995. 5000. 5005. 5010. 5015. 5020. 5025. 5030. 5035. 5040. 5045. 5050. 5055. 5060. 5065. 5070. 5075. 5080. 5085. 5090. 5095. 5100. 5105. 5110. 5115. 5120. 5125. 5130. 5135. 5140. 5145. 5150. 5155. 5160. 5165. 5170. 5175. 5180. 5185. 5190. 5195. 5200. 5205. 5210. 5215. 5220. 5225. 5230. 5235. 5240. 5245. 5250. 5255. 5260. 5265. 5270. 5275. 5280. 5285. 5290. 5295. 5300. 5305. 5310. 5315. 5320. 5325. 5330. 5335. 5340. 5345. 5350. 5355. 5360. 5365. 5370. 5375. 5380. 5385. 5390. 5395. 5400. 5405. 5410. 5415. 5420. 5425. 5430. 5435. 5440. 5445. 5450. 5455. 5460. 5465. 5470. 5475. 5480. 5485. 5490. 5495. 5500. 5505. 5510. 5515. 5520. 5525. 5530. 5535. 5540. 5545. 5550. 5555. 5560. 5565. 5570. 5575. 5580. 5585. 5590. 5595. 5600. 5605. 5610. 5615. 5620. 5625. 5630. 5635. 5640. 5645. 5650. 5655. 5660. 5665. 5670. 5675. 5680. 5685. 5690. 5695. 5700. 5705. 5710. 5715. 5720. 5725. 5730. 5735. 5740. 5745. 5750. 5755. 5760. 5765. 5770. 5775. 5780. 5785. 5790. 5795. 5800. 5805. 5810. 5815. 5820. 5825. 5830. 5835. 5840. 5845. 5850. 5855. 5860. 5865. 5870. 5875. 5880. 5885. 5890. 5895. 5900. 5905. 5910. 5915. 5920. 5925. 5930. 5935. 5940. 5945. 5950. 5955. 5960. 5965. 5970. 5975. 5980. 5985. 5990. 5995. 6000. 6005. 6010. 6015. 6020. 6025. 6030. 6035. 6040. 6045. 6050. 6055. 6060. 6065. 6070. 6075. 6080. 6085. 6090. 6095. 6100. 6105. 6110. 6115. 6120. 6125. 6130. 6135. 6140. 6145. 6150. 6155. 6160. 6165. 6170. 6175. 6180. 6185. 6190. 6195. 6200. 6205. 6210. 6215. 6220. 6225. 6230. 6235. 6240. 6245. 6250. 6255. 6260. 6265. 6270. 6275. 6280. 6285. 6290. 6295. 6300. 6305. 6310. 6315. 6320. 6325. 6330. 6335. 6340. 6345. 6350. 6355. 6360. 6365. 6370. 6375. 6380. 6385. 6390. 6395. 6400. 6405. 6410. 6415. 6420. 6425. 6430. 6435. 6440. 6445. 6450. 6455. 6460. 6465. 6470. 6475. 6480. 6485. 6490. 6495. 6500. 6505. 6510. 6515. 6520. 6525. 6530. 6535. 6540. 6545. 6550. 6555. 6560. 6565. 6570. 6575. 6580. 6585. 6590. 6595. 6600. 6605. 6610. 6615. 6620. 6625. 6630. 6635. 6640. 6645. 6650. 6655. 6660. 6665. 6670. 6675. 6680. 6685. 6690. 6695. 6700. 6705. 6710. 6715. 6720. 6725. 6730. 6735. 6740. 6745. 6750. 6755. 6760. 6765. 6770. 6775. 6780. 6785. 6790. 6795. 6800. 6805. 6810. 6815. 6820. 6825. 6830. 6835. 6840. 6845. 6850. 6855. 6860. 6865. 6870. 6875. 6880. 6885. 6890. 6895. 6900. 6905. 6910. 6915. 6920. 6925. 6930. 6935. 6940. 6945. 6950. 6955. 6960. 6965. 6970. 6975. 6980. 6985. 6990. 6995. 7000. 7005. 7010. 7015. 7020. 7025. 7030. 7035. 7040. 7045. 7050. 7055. 7060. 7065. 7070. 7075. 7080. 7085. 7090. 7095. 7100. 7105. 7110. 7115. 7120. 7125. 7130. 7135. 7140. 7145. 7150. 7155. 7160. 7165. 7170. 7175. 7180. 7185. 7190. 7195. 7200. 7205. 7210. 7215. 7220. 7225. 7230. 7235. 7240. 7245. 7250. 7255. 7260. 7265. 7270. 7275. 7280. 7285. 7290. 7295. 7300. 7305. 7310. 7315. 7320. 7325. 7330. 7335. 7340. 7345. 7350. 7355. 7360. 7365. 7370. 7375. 7380. 7385. 7390. 7395. 7400. 7405. 7410. 7415. 7420. 7425. 7430. 7435 |          |

mixture is heated to 320°-340° F. to evaporate all water therefrom, the remainder of the oil is added to cut the grease to the desired soap concentration, and the diluted grease is cooled to 180°-190° F. and homogenized.

10. A method of producing a grease as defined in claim 6 in which a mixture of mixed acids I, coupling agent, bright stock extract, and part of the solvent-refined neutral oil is charged to a grease-making kettle and heated to 120°-130° F. with agitation, the metal hydroxide is added in concentrated aqueous solution to the heated mixture, the resulting mixture is heated to 210°-220° F. until mixed acids I are neutralized, the mixture is heated 320°-340° F. to evaporate all water therefrom, the remainder of the solvent-refined neutral oil is added

to produce the desired soap concentration in the grease, and the diluted grease is cooled to 180°-190° F. and homogenized.

References Cited in the file of this patent

UNITED STATES PATENTS

2,182,056 Bruson et al. ----- Dec. 5, 1939  
2,588,280 O'Halloran et al. ----- Mar. 4, 1952

OTHER REFERENCES

The Manufacture and Application of Lubricating Greases, Boner, Reinhold Pub. Corp., New York, 1954, pages 138, 139, 443 and 952.